

# UNITED STATES PATENT OFFICE.

GILBERT RIGG, OF PALMERTON, PENNSYLVANIA, ASSIGNOR TO NEW JERSEY ZINC COMPANY, OF NEW YORK, N. Y., A CORPORATION OF NEW JERSEY.

## PROCESS OF RECOVERING SULFUR IN ELEMENTARY FORM FROM PYRITE.

1,103,081.

Specification of Letters Patent.

Patented July 14, 1914.

No Drawing.

Application filed March 27, 1911. Serial No. 617,210.

To all whom it may concern:

Be it known that I, GILBERT RIGG, a subject of the King of Great Britain, residing at Palmerton, county of Carbon, State of Pennsylvania, have invented certain new and useful Improvements in Processes of Recovering Sulfur in Elementary Form from Pyrite; and I do hereby declare the following to be a full, clear, and exact description of the invention, such as will enable others skilled in the art to which it appertains to make and use the same.

This invention relates to a process for recovering sulfur in the elementary form from pyrite,  $FeS_2$ , or from pyritiferous ore, with the conversion of the pyrite into pyrrhotite or magnetic sulfid, the formula for pyrrhotite varying somewhat, being given as  $Fe_7S_8$  to  $Fe_{11}S_{12}$ .

In the usual method of converting pyrite into pyrrhotite, the ore is partially roasted in a current of air, the roasting being stopped when sufficient sulfur has been driven off to effect the desired conversion. If the roasting were continued beyond this point, the pyrrhotite would be converted into non-magnetic ferric oxid.

The objection to converting pyrite into pyrrhotite by partially roasting in a current of air is: that the sulfur is driven off as  $SO_2$ , mixed with large volumes of fire gases, so that the gas mixture is too dilute and too impure to be available for sulfuric acid manufacture. The gas mixture is, therefore, usually delivered into the air and not only is the sulfur wasted, but the gases thus discharged are very injurious to vegetation and cause much trouble. By my method, the sulfur is recovered in the form of elementary sulfur or brimstone, and all loss and nuisance are practically obviated.

In carrying the process into effect, I heat the pyrite or pyritiferous ore in a muffle, or in a shaft, from which the fire gases and air are excluded. At temperatures ranging from 600° C. to 800° C., the pyrite gives up part of its sulfur, which passes over as sulfur vapor, and, leaving the muffle or shaft by suitable exit openings, is recovered in the form of elementary sulfur in a suitable condenser. The pyrite, by this treatment, is converted into pyrrhotite.

A further advantage of this method of treatment is that it is impossible to pass beyond the point of converting the pyrite into pyrrhotite or magnetic sulfid. In the process at present employed, on the contrary, where the ore is roasted in a current of air, it is difficult and, with some ores, practically impossible, to interrupt the operation at the point where sufficient sulfur has been burned off to change the pyrite into pyrrhotite. If the roasting is not continued long enough, a certain amount of non-magnetic pyrite is left unchanged, and if carried too far, non-magnetic ferric oxid is produced, which is equally undesirable from the standpoint of converting the entire mass into pyrrhotite. With my method, the pyrite can only change into pyrrhotite. Further heating has no effect upon it, unless the temperature is carried to such a degree as to fuse the charge, and this is easily obviated. Consequently, the heating can be continued long enough to insure the complete conversion of the pyrite into pyrrhotite without incurring any danger from over-roasting.

Having thus described my invention, what I claim is:

1. The process of converting pyrite into pyrrhotite, which consists in expelling by heat, in the absence of air, a portion of the sulfur from the pyrite at temperatures maintained below the fusion point of the pyrite until the pyrite is converted into pyrrhotite, that is to say, into magnetic sulfid; substantially as described.

2. The process of converting pyrite into pyrrhotite, which consists in expelling by heat in the absence of air, a portion of the sulfur from the pyrite at temperatures maintained below the fusion point of the pyrite until the pyrite is converted into pyrrhotite, that is to say, into magnetic sulfid, said temperatures ranging from 600° C. to 800° C.; substantially as described.

In testimony whereof I affix my signature, in presence of two witnesses.

GILBERT RIGG.

Witnesses:

HENRY HARDENBERGH,  
E. G. TACY.